

# UNITED STATES PATENT OFFICE.

EDGAR L. CULVER, OF AUSTIN, TEXAS.

## FUEL.

1,195,784.

Specification of Letters Patent. Patented Aug. 22, 1916.

No Drawing.

Application filed June 26, 1915. Serial No. 36,495.

To all whom it may concern:

Be it known that I, EDGAR L. CULVER, a citizen of the United States, residing at Austin, in the county of Travis and State of Texas, have invented certain new and useful improvements in Fuel, of which the following is a specification.

My invention relates to an improved fuel and method of manufacturing same from 10 waste material.

The object is not only to produce an improved fuel, but also to utilize the waste or trash of a community, factories, packing-houses, saw-mills, house garbage, solids 15 from sewerage, and garbage of whatever description.

The non-combustible matter, such as cans, iron, glass, stones, and dirt are separated, and the remaining mass is placed in a pul- 20 verizer or reduction machine, where it is ground and reduced to suitable size. It is then conveyed to a pug-mill or other ap- proved mechanism for reducing it to a pulp, water and steam being added so that the 25 mass thus treated becomes a binder sufficient to bind the other ingredients, such as coal or coal-dust which may be added, all to- gether, and the more of a pulp that this mass becomes, the more of the coal or coal 30 dust it will bind solidly together. From the pug-mill or pulping machine, the mass is preferably fed to a mixer, although the mix- 35 ing might be done right in the pug-mill or pulping machine. It is then that the fine coal or coal-dust in suitable proportions—if used—is added. The proportion is deter- 40 mined by the class of fuel required. For instance, if a quick fire is required, less coal dust is used; and at this time might be 45 added, if desired, a small percentage of crude oil, asphaltum or waste pitch from an oil refinery for the purpose of increasing the combustion, and any of the numerous common disinfectants in sufficient amount to 50 kill any infectious germ life is also added; also some of the numerous and well-known deodorizing agents, preferably coal- or water-tar may be added, for the reason that the tar is an additional factor in the de- 55 dorizing of the smoke while the fuel is being consumed. The entire mass, including these ingredients, is then thoroughly mixed, the mixture being reduced to the consistency of that of stiff mud brick material before being 60 molded. The mass is then conveyed to a

molding machine where it is molded into the desired shapes and sizes, and from this molding machine is conveyed to a shed, kiln, or into the open to dry, somewhat as bricks or lumber are dried.

The mass can be conveyed, if desired, from the mixer or pug-mill direct to a dry- 65 ing-room or kiln, and when sufficient mois- ture shall have been removed, it is conveyed direct to a power-press where the mass is 70 pressed into desired shapes and size, and in any case when the composition is dry, it is ready for consumption and storage, and forms an excellent fuel for domestic or other purposes, having the heat units of value of 75 most of the lump coal mined, and it pos- sses the added advantage that it will not deteriorate, or slack to any great extent, re- 80 gardless of how long in storage; and it does not absorb moisture more than common fire- wood.

The fuel is wholly consumed, leaving practically no clinkers, and very little smoke and soot.

Thus it will be seen that the fuel is manu- 85 factured from practically what is now a waste product, and that part which is now considered garbage is not only a waste but an expense for its disposal, and at present a menace to health, and unsanitary.

The invention, therefore, consists in a product composed of certain waste elements, such as garbage, trash, paper, manure, and all materials of a fibrous nature, mixed with hot water or steam, or both, into a binding 90 pulp, to which may be added tar during the pulping of the mass, the steam and tar acting to kill all germ-life, and the tar serving as a deodorizer for the manufactured product, as well as deodorizing the fumes while 95 combustion takes place. The pulp thus formed is conveyed to a pug-mill where the coal (if used) is added, after having been reduced to a dust, and the mass is thor- 100oughly mixed, and then molded and dried. The pulp formed is somewhat in the nature of that used in the manufacture of paste- board, and constitutes an excellent binder.

I claim:

1. The herein-described method of manu- 105 facturing fuel, which consists in forming a binder from a pulp of city refuse, all of which is ground fine and mixed in the pres- ence of liquid heated to a sufficiently high degree to kill germ life therein, and adding 110

a deodorizing agent, which is commingled with the pulp forming a binder, after which the whole mass is dried.

2. The herein-described method of manufacturing fuel, which consists in forming a binder from a pulp of city refuse, all of which is ground fine and mixed in the presence of liquid heated to a sufficiently high

degree to kill germ life therein, adding a deodorizing agent, which is commingled with the pulp forming a binder, then adding carbonaceous material, after which the whole mass is dried.

In testimony whereof I affix my signature.

EDGAR L. CULVER.